

June 11, 1940.

G. EDWARDS

2,203,679

METHOD OF AND APPARATUS FOR MAKING BIMETALLIC STRIP

Filed Dec. 16, 1938

2 Sheets-Sheet 1



Fig. 4

BY

Gray, Oberlin & Gray  
ATTORNEYS

INVENTOR.  
GEORGE EDWARDS

June 11, 1940.

G. EDWARDS

2,203,679

METHOD OF AND APPARATUS FOR MAKING BIMETALLIC STRIP

Filed Dec. 16, 1938 2 Sheets-Sheet 2



Fig. 5



Fig. 6



Fig. 8



Fig. 7

INVENTOR.  
GEORGE EDWARDS

BY

Pray, Oberlin & Pray  
ATTORNEYS.

## UNITED STATES PATENT OFFICE

2,203,679

METHOD OF AND APPARATUS FOR MAKING  
BIMETALLIC STRIPGeorge Edwards, Cleveland, Ohio, assignor to  
The Cleveland Graphite Bronze Company,  
Cleveland, Ohio, a corporation of Ohio

Application December 16, 1938, Serial No. 246,127

6 Claims. (Cl. 22—57.2)

This invention relates, as indicated, to methods of and apparatus for making bimetallic or composite strip, but has reference more particularly to methods and apparatus for the application of one metal in molten condition onto a strip of a second metal of higher melting point. The invention is particularly directed to the problem of applying metal such as a copper alloy having a high melting point to steel strips of such widths as three and one-half inches and greater, while controlling the thickness of the coating alloy, securing a true and uniform bond or weld between the two metals, and preventing undue contamination of the molten metal from remaining in contact with other metals during the operation.

The problem which we have solved by the present invention is obviously far removed from that of applying a thin coating of such low melting point metals as tin, zinc, or alloys of the same to rods, wires and strips, since in such operations which have been commercially practical for some years the molten metal can either be confined by a chamber on the strip, or the strip, rod or the like can be drawn through a bath of the molten metal.

The nature of the problem and the manner in which the control of the aforesaid factors and conditions is best exercised will probably be best understood by a description thereof with reference to actual working conditions, as illustrated, for example, in the accompanying drawings, wherein:

Fig. 1 is a longitudinal cross-sectional view of the pouring box showing the strip moving through the box and having molten bronze or brass applied to the upper surface thereof;

Fig. 2 is a plan view of the pouring box, with the cover removed;

Fig. 3 is a cross-sectional view, taken on the line 3—3 of Fig. 1;

Fig. 4 is a cross-sectional view, taken on the line 4—4 of Fig. 1;

Fig. 5 is a cross-sectional view of apparatus which may be employed for tilting the pouring box;

Fig. 6 is an elevation of the base and carriage of the tilting apparatus;

Fig. 7 is a fragmentary cross-sectional view, taken on the line 7—7 of Fig. 6; and

Fig. 8 is a fragmentary cross-sectional view, taken on the line 8—8 of Fig. 6.

In order to explain clearly the nature of the present invention and the difficulties which are overcome by the use of the present method, it

should be stated that a normal operation in which plastic bronze, for example, is poured onto the steel strip involves the movement of the strip at the rate of, say, 15 feet per minute. The strip, while it may be of any width desired, may be taken, for illustration, at 5 inches. It is designed to put a coating of plastic bronze onto the steel which, when finished, will be .020, .030 or .050 in thickness. To secure this thickness of material on the finished strip it is necessary naturally to produce an initial thickness greater than the finished thickness. The maximum thickness may be set at .100 which, when machined down, will be .060.

The application of a coating of this thickness requires the pouring of only about 10 pounds of metal per minute, which is approximately one ounce of molten metal per inch of length of the strip on which it is poured. The problem which this situation presents is that of pouring an extremely small stream of metal which would represent one ounce of metal per inch of length of the strip, and causing this molten metal to spread laterally the full width of the strip in the time interval during which each portion of the strip is beneath the stream of poured metal. The problem is greatly complicated by the varying degrees of viscosity of the metal which are in turn affected by many different conditions in the apparatus.

This problem has been solved in the present method by pouring the necessarily small stream of molten metal onto the strip from a height very slightly above the surface of the strip so that there will be no spattering of metal, causing a pool of metal to form on the strip which has sufficient depth, that is, head, to cause the metal to flow transversely of the strip to the edges thereof in order to completely coat the strip and at the same time move the strip lengthwise under the poured stream to remove each increment of the strip from beneath the stream with a coating of metal. In effect, the process consists of establishing a pool of molten metal on the strip of sufficient height to insure spreading of the metal laterally across the strip and maintaining this pool at the predetermined height or head by adding molten metal approximately as rapidly to the pool as such metal is removed from the pool by the forward movement of the strip.

It is possible, however, with very narrow strips or with heavy streams of molten metal to secure spreading of the metal all the way across the strip without the formation of any substantial

pool. For example, a strip 1" in width can be coated from the stream without forming any substantial pool, as the metal will spread and flow over such a narrow width even when not 5 under the influence of any substantial head in the form of a pool. It has been found that a pool is, however, necessary where the width of the strip is approximately twenty or more times the thickness of the coating applied to the molten 10 strip, even in cases of narrow strips the application is improved by following the above formula.

Referring more particularly to Figs. 1 to 4 inclusive of the drawings, it will be seen that the pouring box comprises a center guide shoe 1 or base plate 1 having laterally spaced ribs or flanges 2 on the upper surface thereof. Mounted 15 on the base plate 1 is the pouring box proper which comprises a casting having side walls 3 connected at one end by a back wall 4, and at the other end by a front wall or bridging piece 5. The side walls 3 are provided on their lower surfaces with ribs or flanges 6, which are spaced inwardly from the ribs 2 to provide spaces for a purpose to be presently disclosed. The back 20 wall 3 is transversely curved on its lower surface as at 7, and is beveled as at 8, immediately in advance of said curved surface.

Mounted on the side walls 3 of the pouring box is a pan 9, having a transversely curved bottom 10 which slopes rearwardly and downwardly when considered with reference to the direction of movement of the strip. This is further provided with an end wall or spreader plate 11, which is disposed at an acute angle to the strip as the latter moves through the box. This plate 11 extends crosswise of the space between the inner surfaces of the side walls of the box and the bottom 10 terminates short of such spreader plate, so as to leave a space through which the 40 molten metal flows onto the strip. In practice, the lower edge of the spreader plate 11 is about  $\frac{1}{4}$  inch from the strip.

Mounted on the box is a cover 12 which has a circular opening through which the molten metal flows onto the bottom 10 of the pan 9.

Associated with the pouring box is a front guide shoe 13 which is aligned with the center guide shoe 1, and has mounted thereon a cover 14. A rear guide 15 is also provided which is 50 aligned with the opening in the rear of the pouring box.

Before entering the pouring box, the strip S is provided at its edges with flanges F, which serve as means for laterally confining the flow 55 of the applied molten metal. As the strip enters the pouring box, its forward end strikes the beveled surface 8 of the back wall 3 and the strip is thereby directed below the curved surface 7 of the back wall, and is transversely bowed so as to present a concave upper surface to the molten metal subsequently applied thereto. As 60 the strip proceeds through the pouring box, the flanges F thereof move through the spaces between the ribs 2 and 6.

65 The object of this bowing or concaving the strip is to avoid uncontrolled buckling or warping of the strip which might otherwise occur, due to the high temperature to which the strip is heated even before it enters the pouring box.

70 As the concave strip proceeds through the pouring box, molten metal M which may be bronze or brass is poured upon the upper concaved surface thereof, and, due to such concavity of the strip, such molten metal will be 75 thicker in the center than at its lateral edges.

This condition, moreover, is somewhat aggravated due to the surface tension of the metal, which causes the metal to resist lateral spreading.

I have been able to overcome this condition, without confining the molten metal longitudinally of the strip by devices such as the adjustable end gate or wall, to which reference has been made, by causing the strip S to move upwardly and at an angle to the horizontal, the molten metal being poured onto the strip as it 10 is thus inclined. By thus inclining the strip, a pool of molten metal, indicated by the reference numeral P, is formed, and the excess metal at the center of the strip, which is due to the concavity of the strip, will continuously flow rearwardly into this pool from the point at which the strip reassumes a horizontal position, that is, a point somewhat beyond the right end of Fig. 1 15 of the drawings. This rearward flow is primarily a flow due to gravity, and is such that 20 the thickness of the molten metal layer at the point where the strip reassumes a horizontal position will be more or less uniform, that is, the thickness of such metal at the center of the strip will not vary materially from that of the 25 edges of the strip. Moreover, the kinetic energy of such molten metal, as it flows rearwardly into the pool, tends to overcome its surface tension to some extent, thereby improving the distribution effect.

Since the flow of molten metal is constant and uniform in amount, the depth of the pool will depend on the angle of inclination of the strip, and upon the speed of the strip. The speed of the strip is so controlled that the rear edge of the pool P is not permitted to come into contact with the back wall 3 of the pouring box. The pool does not normally come into contact with the front wall 5 of the pouring box, since the latter does not extend downwardly sufficiently to contact the normal pool. The spreader plate 11 is, of course, subject to corrosion due to the molten metal flowing thereover, but since this plate is part of a small casting which is readily removable from the pouring box, it can 45 be replaced at a cost which is but a fraction of the cost of the entire pouring box. There is no appreciable contamination of the molten metal from the metal of the plate 11 since the rate of 50 corrosion of this plate is extremely low.

The extent to which the strip is inclined will vary in accordance with the viscosity of the metal which is applied to the strip, but in general, when working with metals such as plastic bronze and brasses, the pouring box is tilted about 2° to 55 the horizontal at the outset of the pouring operations. After the operations have proceeded for some time and the various temperatures have been more or less equalized, the angle of inclination may be reduced.

Since the viscosity of metals decreases in general as the temperature of the metals increase, the inclination may also be said to be varied in accordance with the temperature of the metal which is applied to the strip.

The pouring box is normally disposed within a furane 20, lined with refractory material 21, and having a cover 22. A conduit 23 extends through the cover 22 and terminates adjacent the lower end 24 of the pouring spout, as shown 70 in Fig. 5. This conduit is for the purpose of introducing a non-oxidizing or reducing gas to the locality where the molten metal is applied to the backing strip S.

For the purpose of tilting the furnace, and 75

consequently the pouring box and associated parts, a carriage 25 is provided which is mounted on rollers 26 journaled in a base 27. The carriage 25 is of substantially rectangular form, and is provided at the four corners thereof with screw jacks 28, upon which the furnace rests, and through suitable manipulation of which the furnace is tilted. The tilting may, however, be accomplished in other ways which will readily occur to those skilled in the art to which the invention relates.

It will be noted that since four screw jacks are provided, one at each corner of the furnace, that the furnace can be inclined transversely as well as longitudinally, and that the strip can accordingly be transversely inclined. This at times is desirable for the purpose of causing the pool of molten metal which is applied to the strip to spread toward the edges of the strip.

20 The surface tension, and consequently the viscosity, of the molten metal may be controlled to some extent by changes in the atmospheric conditions within the pouring box. This may be accomplished, for example, by increasing the hydrogen content of the non-oxidizing or reducing gas which is introduced into the pouring box through the conduit 23. Thus, when the metal becomes sluggish, the hydrogen content of the gas, which is essentially a mixture of nitrogen and hydrogen, may be increased from about 7% up to about 15%.

Specific examples of the methods used for various coating metals are given below. In these examples, steel strip having a thickness of from 35 about .020" to about .135", and containing from about .04% to about .20% carbon was employed.

(1) The strip, after being heated to a temperature of about 1850° F. in a non-oxidizing atmosphere, is passed through the pouring box in the manner described, and is coated with a bronze alloy containing from 55% to 65% copper and from 35% to 45% lead, the temperature of the coating metal being from about 2250° to 2350° F. The strip is inclined at an angle of about 2 degrees to the horizontal.

(2) The strip, after being heated as in example (1) is coated with a bronze alloy containing about 78% copper, 9% to 11% lead and 9% to 11% tin, the temperature of this coating metal being from about 2250° F. to about 2350° F. The angle of inclination of the strip is about 2 degrees.

(3) The strip, after being heated as in example (1) is coated with a brass containing about 60% copper and about 40% zinc, the temperature of the coating metal being about 1800° F. The strip is inclined at an angle of about 2 degrees to the horizontal.

Other coating metals which have been employed are a bronze containing 67%--74% copper, 22%--27% lead, 3%--4% tin and 3% zinc, and another containing 83% copper, 7%--9% lead, 3.5%--4.5% tin and 4% zinc. For these the strip is inclined at an angle of about 2 degrees to the horizontal.

In each case, after the strip is coated, the strip is cooled and the coating solidified, which may be effected by any convenient method, such cooling being effected immediately after the strip emerges from the furnace. The cooling may also be effected by means of air.

It is to be understood, however, that the invention is not in any way limited to the use of any particular base metal or coating metal, nor to any specified thickness of metal. The method is also applicable to the coating of metals such as invar, 5 and to the use of other coating metals, such as aluminum and aluminum alloys. The product may be used for various purposes, such as, for example, bearings, bushings, thermostats, etc.

Other forms may be employed embodying the 10 features of my invention instead of the one herein explained, change being made as regards the means and the steps herein disclosed, provided the elements stated by any of the following claims or the equivalent of such stated elements be employed, whether produced by my preferred method 15 or by others embodying steps equivalent to those stated in the following claims.

I therefore point out and distinctly claim as my invention:

20 1. The method of making a bimetallic strip which consists in continuously moving a metal strip in a direction inclined upwardly to the horizontal, pouring molten metal on said strip to form a pool lying intermediate the edges of the strip, 25 and varying the inclination of the strip to cause spreading of the pool toward the edges of the strip.

2. The method of making a bimetallic strip which consists in continuously moving a metal 30 strip, pouring molten metal on said strip to form a pool lying intermediate the edges of the strip and inclining said strip transversely to cause spreading of the pool toward the edges of the strip.

35 3. The method of making a bimetallic strip which consists in continuously moving a metal strip in a direction inclined upwardly to the horizontal, pouring molten metal on said strip to form a pool lying intermediate the edges of the strip, varying the inclination of the strip and 40 inclining the strip transversely to cause spreading of the pool toward the edges of the strip.

4. The method of making bimetallic strip which consists in continuously moving a metal 45 strip through a pouring box having a rear wall, said pouring box being inclined upwardly in the direction of movement of the strip, applying molten metal to the upper surface of the inclined strip and controlling the forward movement of 50 said strip so as to avoid contact of said molten metal with said rear wall of the pouring box.

5. Apparatus for making a bimetallic strip comprising a pouring box through which said strip is adapted to be passed, said box having an entrance and an exit for said strip and means for elevating said exit relatively to said entrance whereby said strip will pass through the box at an upward inclination, and other means for elevating either side of the pouring box.

60 6. Apparatus for making bimetallic strip comprising a pouring box through which said strip is adapted to be passed, said box having an entrance and an exit for said strip, the exit being elevated relatively to said entrance whereby said strip will pass through the box at an upward 65 inclination, and means for varying said inclination.

GEORGE EDWARDS.